

[54] HYDROCARBON CONVERSION WITH A  
SULFIDED SUPERACTIVE  
MULTIMETALLIC CATALYTIC  
COMPOSITE

[75] Inventor: George J. Antos, Bartlett, Ill.

[73] Assignee: UOP Inc., Des Plaines, Ill.

[\*] Notice: The portion of the term of this patent  
subsequent to Aug. 21, 1996, has  
been disclaimed.

[21] Appl. No.: 45,024

[22] Filed: Jun. 4, 1979

## Related U.S. Application Data

[63] Continuation-in-part of Ser. No. 833,332, Sep. 14, 1977,  
Pat. No. 4,165,276.[51] Int. Cl.<sup>3</sup> ..... C10G 35/08

[52] U.S. Cl. ..... 208/139; 208/138

[58] Field of Search ..... 208/139, 138

## [56] References Cited

## U.S. PATENT DOCUMENTS

4,124,491 11/1978 Antos et al. ..... 208/139  
4,165,276 8/1979 Antos ..... 208/139

Primary Examiner—Curtis R. Davis

Attorney, Agent, or Firm—James R. Hoatson, Jr.;  
Thomas K. McBride; William H. Page, II

## [57] ABSTRACT

Hydrocarbons are converted by contacting them at hydrocarbon conversion conditions with a novel sulfided superactive multimetallic catalytic composite comprising a sulfided combination of a catalytically

effective amount of a pyrolyzed rhenium carbonyl component with a porous carrier material containing a uniform dispersion of catalytically effective amounts of a platinum group component, which is maintained in the elemental metallic state during the incorporation and pyrolysis of the rhenium carbonyl component. In a highly preferred embodiment, this novel catalytic composite also contains a catalytically effective amount of a halogen component. The platinum group component, pyrolyzed rhenium carbonyl component, sulfur component, and optional halogen component are preferably present in the multimetallic catalytic composite in amounts, calculated on an elemental basis, corresponding to about 0.01 to about 2 wt. % platinum group metal, about 0.01 to about 5 wt. % rhenium, 0.001 to about 0.2 wt. % sulfur, and about 0.1 to about 3.5 wt. % halogen. A key feature associated with the preparation of the subject catalytic composite is reaction of a rhenium carbonyl complex with a porous carrier material containing a uniform dispersion of a platinum group component maintained in the elemental state, whereby the interaction of the rhenium moiety with the platinum group moiety is maximized due to the platinophilic (i.e. platinum-seeking) propensities of the carbon monoxide ligands used in the rhenium reagent. A specific example of the type of hydrocarbon conversion process disclosed herein is a process for the catalytic reforming of a low octane gasoline fraction wherein the gasoline fraction and a hydrogen stream are contacted with the subject sulfided superactive multimetallic catalytic composite at reforming conditions.

22 Claims, 3 Drawing Figures

Figure 1



Figure 2



Figure 3



HYDROCARBON CONVERSION WITH A  
SULFIDED SUPERACTIVE MULTIMETALLIC  
CATALYTIC COMPOSITE

CROSS-REFERENCE TO RELATED  
DISCLOSURE

This application is a continuation-in-part of my prior, copending application Ser. No. 833,332 filed Sept. 14, 1977 and issued as U.S. Pat. No. 4,165,276 on Aug. 21, 1979. All of the teachings of this prior application are specifically incorporated herein by reference.

The subject of the present invention is a novel sulfided superactive multimetallic catalytic composite which has remarkably superior activity, selectivity and resistance to deactivation when employed in a hydrocarbon conversion process that requires a catalytic agent having both a hydrogenation-dehydrogenation function and a carbonium ion-forming function. The present invention, more precisely, involves a novel dual-function sulfided superactive multimetallic catalytic composite which quite surprisingly enables substantial improvements in hydrocarbon conversion processes that have traditionally used a platinum group metal-containing, dual-function catalyst. According to another aspect, the present invention comprehends the improved processes that are produced by the use of the instant sulfided superactive platinum-rhenium catalyst system which is characterized by a unique reaction between a rhenium carbonyl component and a porous carrier material containing a uniform dispersion of a platinum group component, which is maintained in the elemental metallic state during the incorporation and pyrolysis of the rhenium carbonyl component, whereby the interaction between the rhenium moiety and the platinum group moiety is maximized on an atomic level. In a specific aspect, the present invention concerns a catalytic reforming process which utilizes the subject sulfided catalyst to markedly improve activity, selectivity and stability characteristics associated therewith to a degree not heretofore realized for a sulfided platinum-rhenium catalyst system. Specific advantages associated with use of the present sulfided superactive platinum-rhenium catalyst system in a catalytic reforming process relative to those observed with the corresponding sulfided prior art sulfided platinum-rhenium catalyst system are: (1) increased ability to make octane at low severity operating conditions; (2) enhanced capability to maximize C<sub>5</sub>+ reformate and hydrogen production; (3) augmented ability to expand the catalyst life before regeneration becomes necessary in conventional temperature-limited catalytic reforming units; (4) increased tolerance to conditions which are known to increase the rate of production of deactivating coke deposits; (5) diminished requirements for amount of catalyst to achieve same results as the prior art catalyst systems at no sacrifice in catalyst life before regeneration; and (6) capability of operating at increased charge rates with the same amount of catalyst and at similar conditions as the prior art catalyst systems without any sacrifice in catalyst life before regeneration.

Composites having a hydrogenation-dehydrogenation function and a carbonium ion-forming function are widely used today as catalysts in many industries, such as the petroleum and petrochemical industry, to accelerate a wide spectrum of hydrocarbon conversion reactions. Generally, the carbonium ion-forming function is thought to be associated with an acid-acting material of

the porous, adsorptive, refractory oxide type which is typically utilized as the support or carrier for a heavy metal component such as the metals or compounds of metals of Groups V through VIII of the Periodic Table to which are generally attributed the hydrogenation-dehydrogenation function.

These catalytic composites are used to accelerate a wide variety of hydrocarbon conversion reactions such as hydrocracking, hydrogenolysis, isomerization, dehydrogenation, hydrogenation, desulfurization, cyclization, polymerization, alkylation, cracking, hydroisomerization, dealkylation, transalkylation, etc. In many cases, the commercial applications of these catalysts are in processes where more than one of the reactions are proceeding simultaneously. An example of this type of process is reforming wherein a hydrocarbon feedstream containing paraffins and naphthenes is subjected to conditions which promote dehydrogenation of naphthenes to aromatics, dehydrocyclization of paraffins to aromatics, isomerization of paraffins and naphthenes, hydrocracking and hydrogenolysis of naphthenes and paraffins, and the like reactions, to produce an octane-rich or aromatic-rich product stream. Another example is a hydrocracking process wherein catalysts of this type are utilized to effect selective hydrogenation and cracking of high molecular weight unsaturated materials, selective hydrocracking of high molecular weight materials, and other like reactions, to produce a generally lower boiling, more valuable output stream. Yet another example is a hydroisomerization process wherein a hydrocarbon fraction which is relatively rich in straight-chain paraffin compounds is contacted with a dual-function catalyst to produce an output stream rich in isoparaffin compounds.

Regardless of the reaction involved or the particular process involved, it is of critical importance that the dual-function catalyst exhibit not only the capability to initially perform its specified functions, but also that it has the capability to perform them satisfactorily for prolonged periods of time. The analytical terms used in the art to measure how well a particular catalyst performs its intended functions in a particular hydrocarbon reaction environment are activity, selectivity, and stability. And for purposes of discussion here, these terms are conveniently defined for a given charge stock as follows: (1) activity is a measure of the catalyst's ability to convert hydrocarbon reactants into products at a specified severity level where severity level means the conditions used—that is, the temperature, pressure, contact time, and presence of diluents such as H<sub>2</sub>; (2) selectivity refers to the amount of desired product or products obtained relative to the amount of reactants charged or converted; (3) stability refers to the rate of change with time of the activity and selectivity parameters—obviously, the smaller rate implying the more stable catalyst. In a reforming process, for example, activity commonly refers to the amount of conversion that takes place for a given charge stock at a specified severity level and is typically measured by octane number of the C<sub>5</sub>+ product stream; selectivity refers to the amount of C<sub>5</sub>+ yield, relative to the amount of the charge, that is obtained at the particular activity or severity level; and stability is typically equated to the rate of change with time of activity, as measured by octane number of C<sub>5</sub>+ product and of selectivity as measured by C<sub>5</sub>+ yield. Actually the last statement is not strictly correct because generally a continuous re-

forming process is run to produce a constant octane C<sub>5</sub>+ product with severity level being continuously adjusted to attain this result; and furthermore, the severity level is for this process usually varied by adjusting the conversion temperature in the reaction so that, in point of fact, the rate of change of activity finds response in the rate of change of conversion temperatures and changes in this last parameter are customarily taken as indicative of activity stability.

As is well known to those skilled in the art, the principal cause of observed deactivation or instability of a dual-function catalyst when it is used in a hydrocarbon conversion reaction is associated with the fact that coke forms on the surface of the catalyst during the course of the reaction. More specifically, in these hydrocarbon conversion processes the conditions utilized typically result in the formation of heavy, high molecular weight, black, solid or semi-solid, carbonaceous material which is a hydrogen-deficient polymeric substance having properties akin to both polynuclear aromatics and graphite. This material coats the surface of the catalyst and thus reduces its activity by shielding its active sites from the reactants. In other words, the performance of this dual-function catalyst is sensitive to the presence of carbonaceous deposits or coke on the surface of the catalyst. Accordingly, the major problem facing workers in this area of the art is the development of more active and/or selective catalytic composites that are not as sensitive to the presence of these carbonaceous materials and/or have the capability to suppress the rate of the formation of these carbonaceous materials on the catalyst. Viewed in terms of performance parameters, the problem is to develop a dual-function catalyst having superior activity, selectivity, and stability characteristics. In particular, for a reforming process the problem is typically expressed in terms of shifting and stabilizing the C<sub>5</sub>+ yield-octane relationship at the lowest possible severity level—C<sub>5</sub>+ yield being representative of selectivity and octane being proportional to activity.

I have now found a dual-function sulfided and attenuated superactive multimetallic catalytic composite which possesses improved activity, selectivity and stability characteristics relative to similar catalysts of the prior art when it is employed in a process for the conversion of hydrocarbons of the type which have heretofore utilized dual-function, platinum group metal-containing catalytic composites such as processes for isomerization, hydroisomerization, dehydrogenation, desulfurization, denitrogenation, hydrogenation, alkylation, hydrodealkylation, disproportionation, polymerization, hydrocyclization, cracking, hydrocracking, halogenation, reforming and the like processes. In particular, I have now established that a sulfided superactive multimetallic catalytic composite, comprising a sulfided combination of a catalytically effective amount of a pyrolyzed rhenium carbonyl component with a porous carrier material containing catalytically effective amounts of a platinum group component, can enable the performance of hydrocarbon conversion processes utilizing dual-function catalysts to be substantially improved if the platinum group component is relatively uniformly dispersed throughout the porous carrier material prior to contact with the rhenium carbonyl reagent, if the oxidation state of the platinum group metal is maintained in the elemental metallic state prior to and during contact with the rhenium carbonyl reagent and if high temperature treatment in the presence of oxygen and/or water

of the resulting reaction product is avoided. A specific example of my discovery involves my finding that a sulfided superactive acidic multimetallic catalytic composite, comprising a sulfided combination of a catalytically effective amount of a pyrolyzed rhenium carbonyl component with a porous carrier material containing a uniform dispersion of catalytically effective amounts of a platinum group component, which is maintained in the elemental metallic state during the incorporation and pyrolysis of the rhenium carbonyl component and of a halogen component, can be utilized to substantially improve the performance of a hydrocarbon reforming process which operates on a low octane gasoline fraction to produce a high octane reformate or aromatic-rich reformate. In the case of a reforming process, some of the major advantages associated with the use of the novel sulfided multimetallic catalytic composite of the present invention include: (1) acquisition of the capability to operate in a stable manner in a high severity operation; for example, a low or moderate pressure reforming process designed to produce a C<sub>5</sub>+ reformate having an octane of at least about 100 F-1 clear; (2) increased average activity for octane upgrading reactions relative to the performance of prior art bimetallic platinum-rhenium catalyst systems as exemplified by the teachings of Kluksdahl in his U.S. Pat. No. 3,415,737; and (3) increased capability to maximize C<sub>5</sub>+ yield and hydrogen production relative to these prior art catalyst systems. In sum, the present invention involves the remarkable finding that carefully controlled sulfiding of a catalyst formed by the addition of a pyrolyzed rhenium carbonyl component to a porous carrier material containing a uniform dispersion of a catalytically effective amount of a platinum group component, which is maintained in the elemental metallic state during the incorporation and pyrolysis of the rhenium carbonyl component, can enable the performance characteristics of the resulting sulfided superactive multimetallic catalytic composite to be sharply and materially improved relative to those associated with the corresponding sulfided prior art platinum-rhenium catalyst system.

It is, accordingly, an object of the present invention to provide a sulfided superactive multimetallic hydrocarbon conversion catalyst having superior performance characteristics relative to the corresponding sulfided prior art platinum-rhenium catalyst systems when utilized in a hydrocarbon conversion process. A second object is to provide a sulfided superactive multimetallic acidic catalyst having dual-function hydrocarbon conversion performance characteristics which are relatively insensitive to the deposition of coke-forming, hydrocarbonaceous materials thereon and to the presence of sulfur contaminants in the reaction environment. A third object is to provide preferred methods of preparation of this sulfided superactive multimetallic catalytic composite which methods insure the achievement and maintenance of its unique properties. Another object is to provide an improved sulfided platinum-rhenium catalyst system having superior activity, selectivity and stability characteristics relative to the sulfided platinum-rhenium catalyst systems of the prior art. Another object is to provide a novel acidic sulfided multimetallic hydrocarbon conversion catalyst which utilizes a pyrolyzed rhenium carbonyl component to beneficially interact with and selectively promote an acidic catalyst containing a halogen component and a uniform dispersion of a platinum group component maintained

in the metallic state during the incorporation and pyrolysis of the rhenium carbonyl component.

Without the intention of being limited by the following explanation, I believe my discovery that rhenium carbonyl can, quite unexpectedly, be used under the circumstances described herein to synthesize an entirely new type of platinum-rhenium catalyst system, is attributable to one or more unusual and unique routes to greater platinum-rhenium interaction that are opened or made available by the novel chemistry associated with the reaction of a rhenium carbonyl reactant with a supported, uniformly dispersed platinum metal. Before considering in detail each of these possible routes to greater platinum-rhenium interaction, it is important to understand that: (1) "platinum" is used herein to mean any one of the platinum group metals; (2) the unexpected results achieved with my catalyst systems are measured relative to the conventional platinum-rhenium catalyst systems as taught in, for example, the Kluksdahl U.S. Pat. No. 3,415,737; (3) the expression "rhenium moiety" is intended to mean the catalytically active form of the rhenium entity derived from the rhenium carbonyl component in the catalyst system; and (4) metallic carbonyls have been suggested generally in the prior art for use in making catalysts such as in U.S. Pat. Nos. 3,591,649; 4,048,110 and 2,798,051, but no one to my knowledge has ever suggested using these reagents in the platinum-rhenium catalyst system, particularly where substantially all of the platinum component of the catalyst is present in a reduced form (i.e. the metal) prior to incorporation of the rhenium carbonyl component. One route to greater platinum-rhenium interaction enabled by the present invention comes from the theory that the effect of rhenium on a platinum catalyst is very sensitive to the particle size of the rhenium moiety; since in my procedure the rhenium is put on the catalyst in a form where it is complexed with carbon monoxide molecules which are known to have a strong affinity for platinum, it is reasonable to assume that when the platinum is widely dispersed on the support, one effect of the CO ligands is to pull the rhenium moiety towards the platinum sites on the catalyst, thereby achieving a dispersion and particle size of the rhenium moiety in the catalyst which closely imitates the corresponding platinum conditions (i.e. this might be called a piggy-back theory). The second route to greater platinum-rhenium interaction is similar to the first and depends on the theory that the effect of rhenium on a platinum catalyst is at a maximum when the rhenium moiety is attached to individual platinum sites; the use of platinophilic CO ligands, as called for by the present invention, then acts to facilitate adsorption or chemisorption of the rhenium moiety on the platinum site so that a substantial portion of the rhenium moiety is deposited or fixed on or near the platinum site where the platinum acts to anchor the rhenium, thereby making it more resistant to sintering at high temperature. The third route to greater platinum-rhenium interaction is based on the theory that the active state for the rhenium moiety in the rhenium-platinum catalyst system is the elemental metallic state and that the best platinum-rhenium interaction is achieved when the proportion of the rhenium in the metallic state is maximized; using a rhenium carbonyl complex to introduce the rhenium into the catalytic composite conveniently ensures availability of more rhenium metal because all of the rhenium in this reagent is present in the elemental metallic state. Another route to greater platinum-rhenium inter-

action is derived from the theory that oxygen at high temperature is detrimental to both the active form of the rhenium moiety (i.e. the metal) and the dispersion of same on the support (i.e. oxygen at high temperatures is suspected of causing sintering of the rhenium moiety); since the catalyst of the present invention is not subject to high temperature treatment with oxygen after rhenium is incorporated, maximum platinum-rhenium interaction is obviously preserved. The final theory for explaining the greater platinum-rhenium interaction associated with the instant catalyst is derived from the idea that the active sites for the platinum-rhenium catalyst are basically platinum metal crystallites that have had their surface enriched in rhenium metal; since the concept of the present invention requires the rhenium to be laid down on the surface of well-dispersed platinum crystallites via a platinophilic rhenium carbonyl complex, the probability of surface enrichment is greatly increased for the present procedure relative to that associated with the random, independent dispersion of both crystallites that has characterized the prior art preparation procedures. It is of course to be recognized that all of these factors may be involved to some degree in the overall explanation of the impressive results associated with my attenuated superactive catalyst system. A further fact to be kept in mind is that the conventional sulfided platinum-rhenium catalyst systems have never been noted for an activity improvement (i.e. the consensus of the art is that they give the same activity as the all platinum catalyst system) but their strong suit has always been very impressive stability; in contrast, my sulfided and attenuated superactive platinum-rhenium catalyst system gives much better average activity than the conventional sulfided platinum-rhenium catalyst system.

Against this background then, the present invention is in one embodiment, a novel multimetallic catalytic composite comprising a sulfided combination of a catalytically effective amount of a pyrolyzed rhenium carbonyl component with a porous material containing a uniform dispersion of catalytically effective amounts of a platinum group component which is maintained in the elemental metallic state during the incorporation and pyrolysis of the rhenium carbonyl component.

In another embodiment, the subject catalytic composite comprises a sulfided combination of a catalytically effective amount of a pyrolyzed rhenium carbonyl component with a porous carrier material containing a catalytically effective amount of a halogen component and a uniform dispersion of catalytically effective amounts of a platinum group component which is maintained in the elemental metallic state during the incorporation and pyrolysis of the rhenium carbonyl component.

In yet another embodiment, the present invention involves a sulfided combination of a pyrolyzed rhenium carbonyl component with a porous carrier material containing a halogen component and a uniform dispersion of a platinum group component which is maintained in the elemental metallic state during the incorporation and pyrolysis of the rhenium carbonyl component, wherein these components are present in amounts sufficient to result in the composite containing, calculated on an elemental basis, about 0.01 to about 2 wt. % platinum group metal, about 0.01 to about 5 wt. % rhenium, about 0.1 to about 3.5 wt. % halogen, and about 0.001 to about 0.2 wt. % sulfur.

In still another embodiment, the present invention comprises any of the catalytic composites defined in the previous embodiments wherein the porous carrier material contains, prior to the addition of the pyrolyzed rhenium carbonyl component, not only a platinum group component but also a catalytically effective amount of a component selected from the group consisting of tin, lead, germanium, cobalt, nickel, iron, zinc, tungsten, chromium, molybdenum, bismuth, indium, gallium, cadmium, tantalum, uranium, copper, silver, gold, one or more of the rare earth metals and mixtures thereof.

In another aspect, the invention is defined as a catalytic composite comprising the sulfided and pyrolyzed reaction product formed by reacting a catalytically effective amount of a rhenium carbonyl complex with a porous carrier material containing a uniform dispersion of catalytically effective amounts of a platinum group metal maintained in the elemental metallic state, subjecting the resulting reaction product to pyrolysis conditions selected to decompose the resulting rhenium carbonyl component and thereafter, contacting the pyrolyzed reaction product with a sulfiding agent at sulfiding conditions.

An ancillary embodiment of the present invention involves a method of preparing any of the catalytic composites defined in the previous embodiments, the method comprising the steps of: (a) reacting a sulfur-containing rhenium carbonyl complex with a porous carrier material containing a uniform dispersion of a platinum group component maintained in the elemental metallic state; (b) subjecting the resulting reaction product to pyrolysis conditions selected to decompose the resulting rhenium carbonyl component, without oxidizing either the platinum group or rhenium components, and to thereby liberate a sulfiding agent; and (c) contacting the pyrolyzed reaction product of step (b) with said sulfiding agent at sulfiding conditions.

A further embodiment involves a process for the conversion of a hydrocarbon which comprises contacting the hydrocarbon and hydrogen with the sulfided superactive catalytic composite defined in any of the previous embodiments at hydrocarbon conversion conditions.

A highly preferred embodiment comprehends a process for reforming a gasoline fraction which comprises contacting the gasoline fraction and hydrogen with the sulfided superactive multimetallic catalytic composites defined in any one of the prior embodiments at reforming conditions selected to produce a high octane reformat.

An especially preferred embodiment is a process for the production of aromatic hydrocarbons which comprises contacting a hydrocarbon fraction rich in aromatic precursors and hydrogen with an acidic catalytic composite comprising a sulfided combination of a catalytically effective amount of a pyrolyzed rhenium carbonyl component with a porous carrier material containing a catalytically effective amount of a halogen component and a uniform dispersion of a catalytically effective amount of a platinum group component maintained in the elemental metallic state during the incorporation and pyrolysis of the rhenium carbonyl component. This contacting is performed at aromatic production conditions selected to produce an effluent stream rich in aromatic hydrocarbons.

Other objects and embodiments of the present invention relate to additional details regarding the essential

and preferred catalytic ingredients, preferred amounts of ingredients, appropriate methods of catalyst preparation, operating conditions for use with the novel catalyst in the various hydrocarbon conversion processes in which it has utility, and the like particulars, which are hereinafter given in the following detailed discussion of each of the essential and preferred features of the present invention.

Considering first the porous carrier material utilized in the present invention, it is preferred that the material be a porous, adsorptive, high surface area support having a surface area of about 25 to about 500 m<sup>2</sup>/g. The porous carrier material should be relatively refractory to the conditions utilized in the hydrocarbon conversion process, and it is intended to include within the scope of the present invention carrier materials which have traditionally been utilized in dual-function hydrocarbon conversion catalysts such as: (1) activated carbon, coke, or charcoal; (2) silica or silica gel, silicon carbide, clays, and silicates including those synthetically prepared and naturally occurring, which may or may not be acid treated for example, attapulgus clay, china clay, diatomaceous earth, fuller's earth, kaolin, kieselguhr, etc., (3) ceramics, porcelain, crushed firebrick, bauxite; (4) refractory inorganic oxides such as alumina, titanium dioxide, zirconium dioxide, chromium oxide, beryllium oxide, vanadium oxide, cesium oxide, hafnium oxide, zinc oxide, magnesia, boria, thoria, silica-alumina, silica-magnesia, chromia-alumina, alumina-boria, silica-zirconia, etc.; (5) crystalline zeolitic aluminosilicates such as naturally occurring or synthetically prepared mordenite and/or faujasite, either in the hydrogen form or in a form which has been treated with multivalent cations; (6) spinels such as MgAl<sub>2</sub>O<sub>4</sub>, FeAl<sub>2</sub>O<sub>4</sub>, ZnAl<sub>2</sub>O<sub>4</sub>, CaAl<sub>2</sub>O<sub>4</sub>, and other like compounds having the formula MO-Al<sub>2</sub>O<sub>3</sub> where M is a metal having a valence of 2; and (7) combinations of elements from one or more of these groups. The preferred porous carrier materials for use in the present invention are refractory inorganic oxides, with best results obtained with an alumina carrier material. Suitable alumina materials are the crystalline aluminas known as gamma-, eta-, and theta-alumina, with gamma- or eta-alumina giving best results. In addition, in some embodiments the alumina carrier material may contain minor proportions of other well known refractory inorganic oxides such as silica, zirconia, magnesia, etc.; however, the preferred support is substantially pure gamma- or eta-alumina. Preferred carrier materials have an apparent bulk density of about 0.3 to about 0.8 g/cc and surface area characteristics (B.E.T.) such that the average pore diameter is about 20 to 300 Angstroms, the pore volume is about 0.1 to about 1 cc/g and the surface area is about 100 to about 500 m<sup>2</sup>/g. In general, best results are typically obtained with a gamma-alumina carrier material which is used in the form of spherical particles having a relatively small diameter (i.e. typically about 1/16 inch), an apparent bulk density of about 0.3 to about 0.8 g/cc, a pore volume (B.E.T.) of about 0.4 to about 0.6 cc/g and a surface area (B.E.T.) of about 150 to about 250 m<sup>2</sup>/g.

The preferred alumina carrier material may be prepared in any suitable manner and may be synthetically prepared or natural occurring. Whatever type of alumina is employed, it may be activated prior to use by one or more treatments including drying, calcination, steaming, etc., and it may be in a form known as activated alumina, activated alumina of commerce, porous

alumina, alumina gel, etc. For example, the alumina carrier may be prepared by adding a suitable alkaline reagent, such as ammonium hydroxide, to a salt of aluminum such as aluminum chloride, aluminum nitrate, etc., in an amount to form an aluminum hydroxide gel which upon drying and calcining is converted to alumina. The alumina carrier may be formed in any desired shape such as spheres, pills, cakes, extrudates, powders, granules, tablets, etc., and utilized in any desired size. For the purpose of the present invention a particularly preferred form of alumina is the sphere, and alumina spheres may be continuously manufactured by the well known oil drop method which comprises: forming an alumina hydrosol by any of the techniques taught in the art and preferably by reacting aluminum metal with hydrochloric acid, combining the resultant hydrosol with a suitable gelling agent and dropping the resultant mixture into an oil bath maintained at elevated temperatures. The droplets of the mixture remain in the oil bath until they set and form hydrogel spheres. The spheres are then continuously withdrawn from the oil bath and typically subjected to specific aging treatments in oil and an ammoniacal solution to further improve their physical characteristics. The resulting aged and gelled particles are then washed and dried at a relatively low temperature of about 300° F. to about 400° F. and subjected to a calcination procedure at a temperature of about 850° F. to about 1300° F. for a period of about 1 to about 20 hours. This treatment effects conversion of the alumina hydrogel to the corresponding crystalline gamma-alumina. See the teachings of U.S. Pat. No. 2,620,314 for additional details.

Another particularly preferred alumina carrier material is synthesized from a unique crystalline alumina powder which has been characterized in U.S. Pat. Nos. 3,852,190 and 4,012,313 as a byproduct from a Ziegler higher alcohol synthesis reaction as described in Ziegler's U.S. Pat. No. 2,892,858. For purposes of simplification, the name "Ziegler alumina" is used herein to identify this material. It is presently available from the Conoco Chemical Division of Continental Oil Company under the trademark Catapal. This material is an extremely high purity alpha-alumina monohydrate (boehmite) which after calcination at a high temperature has been shown to yield a high purity gamma-alumina. It is commercially available in three forms: (1) Catapal SB—a spray dried powder having a typical surface area of 250 m<sup>2</sup>/g; (2) Catapal NG—a rotary kiln dried alumina having a typical surface area of 180 m<sup>2</sup>/g; and (3) Dispal M—a finely divided dispersible product having a typical surface area of about 185 m<sup>2</sup>/g. For purposes of the present invention, the preferred starting material is the spray dried powder, Catapal SB. This alpha-alumina monohydrate powder may be formed into a suitable catalyst material according to any of the techniques known to those skilled in the catalyst carrier material forming art. Spherical carrier material particles can be formed, for example, from this Ziegler alumina by: (1) converting the alpha-alumina monohydrate powder into an alumina sol by reaction with a suitable peptizing agent and water and thereafter dropping a mixture of the resulting sol and a gelling agent into an oil bath to form spherical particles of an alumina gel which are easily converted to a gamma-alumina carrier material by known methods; (2) forming an extrudate from the powder by established methods and thereafter rolling the extrudate particles on a spinning disc until spherical particles are formed which can then be dried

and calcined to form the desired particles of spherical carrier material; and (3) wetting the powder with a suitable peptizing agent and thereafter rolling particles of the powder into spherical masses of the desired size in much the same way that children have been known to make parts of snowmen by rolling snowballs down hills covered with wet snow. This alumina powder can also be formed in any other desired shape or type of carrier material known to those skilled in the art such as rods, pills, pellets, tablets, granules, extrudates and the like forms by methods well known to the practitioners of the catalyst carrier material forming art. The preferred type of carrier material for the present invention is a cylindrical extrudate having a diameter of about 1/32" to about 1/8" (especially about 1/16") and a length to diameter (L/D) ratio of about 1:1 to about 5:1, with a L/D ratio of about 2:1 being especially preferred. The especially preferred extrudate form of the carrier material is preferably prepared by mixing the alumina powder with water and a suitable peptizing agent such as nitric acid, acetic acid, aluminum nitrate and the like material until an extrudable dough is formed. The amount of water added to form the dough is typically sufficient to give a loss on ignition (LOI) at 500° C. of about 45 to 65 wt. %, with a value of about 55 wt. % being especially preferred. On the other hand, the acid addition rate is generally sufficient to provide about 2 to 7 wt. % of the volatile free alumina powder used in the mix, with a value of about 3 to 4% being especially preferred. The resulting dough is then extruded through a suitably sized die to form extrudate particles. These particles are then dried at a temperature of about 500° to 800° F. for a period of about 0.1 to about 5 hours and thereafter calcined at a temperature of about 900° F. to about 1500° F. for a period of about 0.5 to about 5 hours to form the preferred extrudate particles of the Ziegler alumina carrier material. In addition, in some embodiments of the present invention the Ziegler alumina carrier material may contain minor proportions of other well known refractory inorganic oxides such as silica, titanium dioxide, zirconium dioxide, chromium oxide, beryllium oxide, vanadium oxide, cesium oxide, hafnium oxide, zinc oxide, iron oxide, cobalt oxide, magnesia, boria, thoria, and the like materials which can be blended into the extrudable dough prior to the extrusion of same. In the same manner crystalline zeolitic aluminosilicates such as naturally occurring or synthetically prepared mordenite and/or faujasite, either in the hydrogen form or in a form which has been treated with a multivalent cation, such as a rare earth, can be incorporated into this carrier material by blending finely divided particles of same into the extrudable dough prior to extrusion of same. A preferred carrier material of this type is substantially pure Ziegler alumina having an apparent bulk density (ABD) of about 0.6 to 1 g/cc (especially an ABD of about 0.7 to about 0.85 g/cc), a surface area (B.E.T.) of about 150 to about 280 m<sup>2</sup>/g (preferably about 185 to about 235 m<sup>2</sup>/g), and a pore volume (B.E.T.) of about 0.3 to about 0.8 cc/g.

A first essential ingredient of the subject catalyst is the platinum group component. That is, it is intended to cover the use of platinum, iridium, osmium, ruthenium, rhodium, palladium, or mixtures thereof as a first component of the attenuated superactive catalytic composite. It is an essential feature of the present invention that substantially all of this platinum group component is uniformly dispersed throughout the porous carrier material in the elemental metallic state during the incorpo-

ration and pyrolysis of the rhenium carbonyl ingredient. Generally, the amount of this component present in the form of catalytic composites is small and typically will comprise about 0.01 to about 2 wt. % of final catalytic composite, calculated on an elemental basis. Excellent results are obtained when the catalyst contains about 0.05 to about 1 wt. % of platinum, iridium, rhodium, palladium or ruthenium metal. Particularly preferred mixtures of these platinum group metals preferred for use in the composite of the present invention are: (1) platinum and iridium, (2) platinum and rhodium, and (3) platinum and ruthenium.

This platinum group component may be incorporated into the porous carrier material in any suitable manner known to result in a relatively uniform distribution of this component in the carrier material such as coprecipitation or cogelation, ion-exchange or impregnation. The preferred method of preparing the catalyst involves the utilization of a soluble, decomposable compound of platinum group metal to impregnate the carrier material in a relatively uniform manner. For example, this component may be added to the support by commingling the latter with an aqueous solution of chloroplatinic or chloroiridic or chloropalladic acid. Other water-soluble compounds or complexes of platinum group metals may be employed in impregnation solutions and include ammonium chloroplatinate, bromoplatinic acid, platinum trichloride, platinum tetrachloride hydrate, platinum dichlororocarbonyl dichloride, ditnitrodiaminoplatinum, sodium tetranitroplatinate (II), palladium chloride, palladium nitrate, palladium sulfate, diamminepalladium (II) hydroxide, tetramminepalladium (II) chloride, hexamminerhodium chloride, rhodium carbonylchloride, rhodium trichloride hydrate, rhodium nitrate, sodium hexachlororhodate (III), sodium hexanitrorhodate (III), iridium tribromide, iridium dichloride, iridium tetrachloride, sodium hexanitroiridate (III), potassium or sodium chloroiridate, potassium rhodium oxalate, etc. The utilization of a platinum, iridium, rhodium, or palladium chloride compound, such as chloroplatinic, chloroiridic, or chloropalladic acid or rhodium trichloride hydrate, is preferred since it facilitates the incorporation of both the platinum group component and at least a minor quantity of the preferred halogen component in a single step. Hydrogen chloride or the like acid is also generally added to the impregnation solution in order to further facilitate the incorporation of the halogen component and the uniform distribution of the metallic components throughout the carrier material. In addition, it is generally preferred to impregnate the carrier material after it has been calcined in order to minimize the risk of washing away the valuable platinum group compound.

It is especially preferred to incorporate a halogen component into the platinum group metal-containing porous carrier material prior to the reactions thereof with the rhenium carbonyl reagent. Although the precise form of the chemistry of the association of the halogen component with this carrier material is not entirely known, it is customary in the art to refer to the halogen component as being combined with the carrier material or with the platinum group component in the form of the halide (e.g. as the chloride). This combined halogen may be either fluorine, chlorine, iodine, bromine, or mixtures thereof. Of these, fluorine and, particularly, chlorine are preferred for the purposes of the present invention. The halogen may be added to the carrier material in any suitable manner, either during

preparation of the support or before or after the addition of the platinum group component. For example, the halogen may be added, at any stage of the preparation of the carrier material or to the calcined carrier material, as an aqueous solution of a suitable, decomposable halogen-containing compound such as hydrogen fluoride, hydrogen chloride, hydrogen bromide, ammonium chloride, etc. The halogen component or a portion thereof, may be combined with the carrier material during the impregnation of the latter with the platinum group and/or zinc component, for example, through the utilization of a mixture of chloroplatinic acid and hydrogen chloride. In another situation, the alumina hydrosol which is typically utilized to form a preferred alumina carrier material may contain halogen and thus contribute at least a portion of the halogen component to the final composite. For reforming, the halogen will be typically combined with the carrier material in an amount sufficient to result in a final composite that contains about 0.1 to about 3.5%, and preferably about 0.5 to about 1.5%, by weight of halogen, calculated on an elemental basis. In isomerization or hydrocracking embodiments, it is generally preferred to utilize relatively larger amounts of halogen in the catalyst—typically, ranging up to about 10 wt. % halogen calculated on an elemental basis, and more preferably, about 1 to about 5 wt. %. It is to be understood that the specified level of halogen component in the instant sulfided superactive catalyst can be achieved or maintained during use in the conversion of hydrocarbons by continuously or periodically added to the reaction zone a decomposable halogen-containing compound such as an organic chloride (e.g. ethylene dichloride, carbon tetrachloride, t-butyl chloride) in an amount of about 1 to 100 wt. ppm. of the hydrocarbon feed, and preferably about 1 to 10 wt. ppm.

After the platinum group is combined with the porous carrier material, the resulting platinum group metal-containing carrier material will generally be dried at a temperature of about 200° F. to about 600° F. for a period of typically about 1 to about 24 hours or more and thereafter oxidized at a temperature of about 700° F. to about 1100° F. in an air or oxygen atmosphere for a period of about 0.5 to about 10 or more hours sufficient to convert substantially all of the platinum group component to the corresponding platinum group metal oxide. When the preferred halogen component is utilized in the present composition, best results are generally obtained when the halogen content of the platinum group metal-containing carrier material is adjusted during at least a portion of this oxidation step by including a halogen or a halogen-containing compound in the air or oxygen atmosphere utilized. For purposes of the present invention, the particularly preferred halogen is chlorine and it is highly recommended that the halogen compound utilized in this halogenation step be either hydrochloric acid or a hydrochloric acid-producing substance. In particular, when the halogen component of the catalyst is chlorine, it is preferred to use a molar ratio of H<sub>2</sub>O to HCl of about 5:1 to about 100:1 during at least a portion of this oxidation step in order to adjust the final chlorine content of the catalyst to a range of about 0.1 to about 3.5 wt. %. Preferably, the duration of this halogenation step is about 1 to 5 or more hours.

A crucial feature of the present invention involves subjecting the resulting oxidized, platinum group metal-containing, and typically halogen-treated, carrier material to a substantially water-free reduction step before

the incorporation of the rhenium component by means of the rhenium carbonyl reagent. The importance of this reduction step comes from my observation that when an attempt is made to prepare the instant catalytic composite without first reducing the platinum group component, no significant improvement in the platinum-rhenium catalyst system is obtained. Put another way, it is my finding that it is essential for the platinum group component to be well dispersed in the porous carrier material in the elemental metallic state during the incorporation of the rhenium component by the unique procedure of the present invention in order for synergistic interaction of the rhenium carbonyl component with the dispersed platinum group metal to occur according to the theories that I have previously explained. Accordingly, this reduction step is designed to reduce substantially all of the platinum group component to the elemental metallic state and to assure a relatively uniform and finely divided dispersion of this metallic component throughout the porous carrier material. Preferably a substantially pure and dry hydrogen stream (by the use of the word "dry" I mean that it contains less than 20 vol. ppm. water and preferably less than 5 vol. ppm. water) is used as the reducing agent in this step. The reducing agent is contacted with the oxidized, platinum group metal-containing carrier material at conditions including a reduction temperature of about 450° F. to about 1200° F., a gas hourly space velocity (GHSV) sufficient to rapidly dissipate any local concentration of water formed during reduction of the platinum group metal oxide, and a period of about 0.5 to about 10 or more hours selected to reduce substantially all of the platinum group component to the elemental metallic state. Once this condition of finely divided dispersed platinum group metal in the porous carrier material is achieved, it is important that environments and/or conditions that could disturb or change this condition be avoided; specifically, I much prefer to maintain the freshly reduced carrier material containing the uniformly dispersed platinum group metal under a blanket of inert gas to avoid any possibility of contamination of same either by water or by oxygen.

A second essential ingredient of the present attenuated superactive catalytic composite is a rhenium component which I have chosen to characterize as a pyrolyzed rhenium carbonyl component in order to emphasize that the rhenium moiety of interest in my invention is the rhenium produced by decomposing a rhenium carbonyl complex in the presence of a finely divided dispersion of a platinum group metal and in the absence of materials such as oxygen or water could interfere with the basic desired interaction of the rhenium carbonyl component with the platinum group metal component as previously explained. This rhenium component may be utilized in the resulting composite in any amount that is catalytically effective with the preferred amount typically corresponding to about 0.01 to about 5 wt. % thereof, calculated on an elemental rhenium basis. Best results are ordinarily obtained with about 0.05 to about 1 wt. % rhenium. The traditional rule for rhenium-platinum catalyst system is that best results are achieved when the amount of the rhenium component is set as a function of the amount of the platinum group component also hold for my composition; specifically, I find that best results with a rhenium to platinum group metal atomic ratio of about 0.1:1 to about 10:1, with an especially useful range comprising about 0.2:1 to about 5:1 and with superior results achieved at an atomic ratio

of rhenium to platinum group metal of about 1:1 to about 3:1.

The rhenium carbonyl ingredient may be reacted with the reduced platinum group metal-containing porous carrier material in any suitable manner known to those skilled in the catalyst formulation art which results in relatively good contact between the rhenium carbonyl complex and the platinum group component contained in the porous carrier material. One acceptable procedure for incorporating the rhenium carbonyl compound into the composite involves sublimating the rhenium carbonyl complex under conditions which enable it to pass into the vapor phase without being decomposed and thereafter contacting the resulting rhenium carbonyl sublimate with the platinum group metal-containing porous carrier material under conditions designed to achieve intimate contact of the rhenium carbonyl reagent with the platinum group metal dispersed on the carrier material. Typically this procedure is performed under vacuum at a temperature of about 70° to about 250° F. for a period of time sufficient to react the desired amount of rhenium with the carrier material. In some cases, an inert carrier gas such as nitrogen can be admixed with the rhenium carbonyl sublimate in order to facilitate the intimate contacting of same with the metal-containing porous carrier material. A particularly preferred way of accomplishing this rhenium carbonyl reaction step is an impregnation procedure wherein the platinum-loaded porous carrier material is impregnated with a suitable solution containing the desired quantity of the rhenium carbonyl complex. For purposes of the present invention, organic solutions are preferred, although any suitable solution may be utilized as long as it does not interact with the rhenium carbonyl and cause decomposition of same. Obviously the organic solution should be anhydrous in order to avoid detrimental interaction of water with the rhenium carbonyl complex. Suitable solvents are any of the commonly available organic solvents such as one of the available ethers, alcohols, ketones, aldehydes, paraffins, naphthenes and aromatic hydrocarbons, for example, acetone, acetyl acetone, benzaldehyde, pentane, hexane, carbon tetrachloride, methyl isopropyl ketone, benzene, n-butylether, diethyl ether, ethylene glycol, methyl isobutyl ketone, diisobutyl ketone and the like organic solvents. Best results are ordinarily obtained when the solvent is acetone; consequently, the preferred impregnation solution is a rhenium carbonyl complex dissolved in anhydrous acetone. The rhenium carbonyl complex suitable for use in the present invention may be either the pure rhenium carbonyl itself or a substituted rhenium carbonyl such as the rhenium carbonyl halides including the chlorides, bromides, and iodides and the like substituted rhenium carbonyl complexes. After impregnation of the carrier material with the rhenium carbonyl component, it is important that the solvent be removed or evaporated from the catalyst prior to decomposition of the rhenium carbonyl component by means of the hereinafter described pyrolysis step. The reason for removal of the solvent is that I believe that the presence of organic materials such as hydrocarbons or derivatives of hydrocarbons during the rhenium carbonyl pyrolysis step is highly detrimental to the synergistic interaction associated with the present invention. This solvent is removed by subjecting the rhenium carbonyl impregnated carrier material to a temperature of about 100° F. to about 250° F. in the presence of an inert gas or under a vacuum condition until

substantially no further solvent is observed to come off the impregnated material. In the preferred case where acetone is used as the impregnation solvent, this drying of the impregnated carrier material typically takes about one half hour at a temperature of about 225° F. under moderate vacuum conditions.

After the rhenium carbonyl component is incorporated into the platinum-loaded porous carrier material, the resulting composite is, pursuant to the present invention, subjected to pyrolysis conditions designed to decompose substantially all of the rhenium carbonyl material, without oxidizing either the platinum group or the decomposed rhenium carbonyl component. This step is preferably conducted in an atmosphere which is substantially inert to the rhenium component such as in a nitrogen- or noble gas-containing atmosphere. Preferably, this pyrolysis step takes place in the presence of a substantially pure and dry hydrogen stream. It is of course within the scope of the present invention to conduct the pyrolysis step under vacuum conditions. It is much preferred to conduct this step in the substantial absence of free oxygen and substances that could yield free oxygen under the conditions selected. Likewise, it is clear that best results are obtained when this step is performed in the total absence of water and of hydrocarbons and other organic materials. I have obtained best results in pyrolyzing the rhenium carbonyl component while using an anhydrous hydrogen stream at pyrolysis conditions including a temperature of about 300° F. to about 900° F. or more, preferably about 400° F. to about 750° F., a gas hourly space velocity of about 250 to about 1500 hr.<sup>-1</sup> for a period of about 0.5 to about 5 or more hours until no further evolution of carbon monoxide is noted.

An essential feature of the present invention is that the resulting pyrolyzed catalytic composite is subjected to a presulfiding step designed to incorporate sulfur in the form of sulfide into the catalytic composite in an amount, calculated on an elemental basis, corresponding to about 0.001 to about 0.2 wt. % sulfur, and especially about 0.005 to about 0.1 wt. % sulfur. Despite the fact that the precise form of the chemistry of the association of this sulfide component with the catalytic composite is not entirely known, it is customary in the art to refer to the sulfide component as being physically and/or chemically combined with the carrier material and/or with the platinum group and rhenium components in the form of sulfide. This sulfided state can be achieved by contacting the resulting pyrolyzed catalytic composite with a suitable sulfiding agent at appropriate sulfiding conditions selected to result in a sulfide sulfur content within the ranges previously specified. The sulfiding agent is preferably a suitable decomposable sulfur-containing compound such as hydrogen sulfide, lower molecular weight mercaptans, organic sulfides, etc. Preferably, this procedure comprises treating the pyrolyzed catalyst with a sulfiding agent such as a mixture of hydrogen sulfide and a diluent gas such as nitrogen or hydrogen at sulfiding conditions sufficient to effect the desired incorporation of sulfur, generally including a pressure of about 0.1 to about 10 atmospheres, a temperature ranging from about 50° F. up to about 1000° F., and a contact time of about 0.1 to 2 or more hours. It is generally a preferred practice to perform this presulfiding step under substantially water-free and oxygen-free conditions. It is within the scope of the present invention to maintain or achieve the sulfided state of the present catalyst during use in the conversion

of hydrocarbons by continuously or periodically adding a suitable sulfiding agent to the reactor containing the sulfided and attenuated superactive catalyst in an amount sufficient to provide about 1 to 500 wt. ppm., preferably about 1 to about 20 wt. ppm. of sulfur, based on hydrocarbon charge. According to an especially preferred mode of operation, this sulfiding step may be accomplished during the pyrolysis step by utilizing a rhenium carbonyl reagent which has a sulfur-containing ligand or by adding H<sub>2</sub>S to the hydrogen stream which is preferably used therein, during the latter portion of the pyrolysis step.

In embodiments of the present invention wherein the instant sulfided superactive multimetallic catalytic composite is used for the dehydrogenation of dehydrogenatable hydrocarbons or for the hydrogenation of hydrogenatable hydrocarbons, it is ordinarily a preferred practice to include an alkali or alkaline earth metal component in the composite before addition of the rhenium carbonyl component and to minimize or eliminate the preferred halogen component. More precisely, this optional ingredient is selected from the group consisting of the compounds of the alkali metals—cesium, rubidium, potassium, sodium, and lithium—and the compounds of the alkaline earth metals—calcium, strontium, barium, and magnesium. Generally, good results are obtained in these embodiments when this component constitutes about 0.1 to about 5 wt. % of the composite, calculated on an elemental basis. This optional alkali or alkaline earth metal component can be incorporated into the composite in any of the known ways, with impregnation with an aqueous solution of a suitable watersoluble, decomposable compound being preferred.

An optional ingredient for the sulfided and superactive multimetallic catalyst of the present invention is a Friedel-Crafts metal halide component. This ingredient is particularly useful in hydrocarbon conversion embodiments of the present invention wherein it is preferred that the catalyst utilized has a strong acid or cracking function associated therewith—for example, an embodiment wherein the hydrocarbons are to be hydrocracked or isomerized with the catalyst of the present invention. Suitable metal halides of the Friedel-Crafts type include aluminum chloride, aluminum bromide, ferric chloride, ferric bromide, zinc chloride, and the like compounds, with the aluminum halides and particularly aluminum chloride ordinarily yielding best results. Generally, this optional ingredient can be incorporated into the composites of the present invention by any of the conventional methods for adding metallic halides of this type and either prior to or after the rhenium carbonyl reagent is added thereto; however, best results are ordinarily obtained when the metallic halides is sublimed onto the surface of the carrier material after the rhenium carbonyl component is added thereto according to the preferred method disclosed in U.S. Pat. No. 2,999,074. The component can generally be utilized in any amount which is catalytically effective, with a value selected from the range of about 1 to about 100 wt. % of the carrier material generally being preferred.

According to the present invention, a hydrocarbon charge stock and hydrogen are contacted with the instant sulfided superactive multimetallic catalyst in a hydrocarbon conversion zone. This contacting may be accomplished by using the catalyst in a fixed bed system, a moving bed system, a fluidized bed system, or in a batch type operation; however, in view of the danger

of attrition losses of the valuable catalyst and of well known operational advantages, it is preferred to use either a fixed bed system or a dense-phase moving bed system such as is shown in U.S. Pat. No. 3,725,249. It is also contemplated that the contacting step can be performed in the presence of a physical mixture of particles of the catalyst of the present invention and particles of a conventional dual-function catalyst of the prior art. In a fixed bed system, a hydrogenrich gas and the charge stock are preheated by any suitable heating means to the desired reaction temperature and then are passed into a conversion zone containing a fixed bed to the sulfided and attenuated superactive multimetallic catalyst. It is, of course, understood that the conversion zone may be one or more separate reactors with suitable means therebetween to ensure that the desired conversion temperature is maintained at the entrance to each reactor. It is also important to note that the reactants may be contacted with the catalyst bed in either upward, downward, or radial flow fashion with the latter being preferred. In addition, the reactants may be in the liquid phase, a mixed liquid-vapor phase, or a vapor phase when they contact the catalyst, with best results obtained in the vapor phase.

In the case where the sulfided and superactive multimetallic catalyst of the present invention is used in a reforming operation, the reforming system will typically comprise a reforming zone containing one or more fixed beds or dense-phase moving beds of the catalysts. In a multiple bed system, it is, of course, within the scope of the present invention to use the present catalyst in less than all of the beds with a conventional dual-function catalyst being used in the remainder of the beds. This reforming zone may be one or more separate reactors with suitable heating means therebetween to compensate for the endothermic nature of the reactions that take place in each catalyst bed. The hydrocarbon feed stream that is charged to this reforming system will comprise hydrocarbon fractions containing naphthenes and paraffins that boil within the gasoline range. The preferred charge stocks are those consisting essentially of naphthenes and paraffins, although in some cases aromatics and/or olefins may also be present. This preferred class includes straight run gasolines, natural gasolines, synthetic gasolines, partially reformed gasolines, and the like. On the other hand, it is frequently advantageous to charge thermally or catalytically cracked gasolines or higher boiling fractions thereof. Mixtures of straight run and cracked gasolines can also be used to advantage. The gasoline charge stock may be a full boiling gasoline having an initial boiling point of from about 50° F. to about 150° F. and an end boiling point within the range of from about 325° F. to about 425° F., or may be a selected fraction thereof which generally will be a higher boiling fraction commonly referred to as a heavy naphtha—for example, a naphtha boiling in the range of C<sub>7</sub> to 400° F. In some cases, it is also advantageous to charge pure hydrocarbons or mixtures of hydrocarbons that have been extracted from hydrocarbon distillates—for example, straightchain paraffins—which are to be converted to aromatics. It is preferred that these charge stocks be treated by conventional catalytic pretreatment methods such as hydrorefining, hydrotreating, hydrodesulfurization, etc., to remove substantially all sulfurous, nitrogenous, and water-yielding contaminants therefrom and to saturate any olefins that may be contained therein.

In other hydrocarbon conversion embodiments, the charge stock will be of the conventional type customarily used for the particular kind of hydrocarbon conversion being effected. For example, in a typical isomerization embodiment, the charge stock can be a paraffinic stock rich in C<sub>4</sub> to C<sub>8</sub> normal paraffins, or a normal butane-rich stock, or an n-hexane-rich stock, or a mixture of xylene isomers, or an olefin-containing stock, etc. In a dehydrogenation embodiment, the charge stock can be any of the known dehydrogenatable hydrocarbons such as an aliphatic compound containing 2 to 30 carbon atoms per molecule, a C<sub>4</sub> to C<sub>30</sub> normal paraffin, a C<sub>8</sub> to C<sub>12</sub> alkylaromatic, a naphthene, and the like. In hydrocracking embodiments, the charge stock will be typically a gas oil, heavy cracked cycle oil, etc. In addition, alkylaromatics, olefins, and naphthenes can be conveniently isomerized by using the catalyst of the present invention. Likewise, pure hydrocarbons or substantially pure hydrocarbons can be converted to more valuable products by using the sulfided superactive catalyst of the present invention in any of the hydrocarbon conversion processes, known to the art, that use a dual-function catalyst.

In a reforming embodiment, it is generally preferred to utilize the sulfided superactive multimetallic catalytic composite in a substantially water-free environment. Essential to the achievement of this condition in the reforming zone is the control of the water level present in the charge stock and the hydrogen stream which is being charged to the zone. Best results are ordinarily obtained when the total amount of water entering the conversion zone from any sources is held to a level less than 50 ppm. and preferably less than 20 ppm. expressed as weight of equivalent water in the charge stock. In general, this can be accomplished by careful control of the water present in the charge stock and in the hydrogen stream. The charge stock can be dried by using any suitable drying means known to the art, such as a conventional solid adsorbent having a high selectivity for water, for instance, sodium or calcium crystalline aluminosilicates, silica gel, activated alumina, molecular sieves, anhydrous calcium sulfate, high surface area sodium, and the like adsorbents. Similarly, the water content of the charge stock may be adjusted by suitable stripping operations in a fractionation column or like device. And in some cases, a combination of adsorbent drying and distillation drying may be used advantageously to effect almost complete removal of water from the charge stock. In an especially preferred mode of operation, the charge stock is dried to a level corresponding to less than 5 wt. ppm. of water equivalent. In general, it is preferred to maintain the hydrogen stream entering the hydrocarbon conversion zone at a level of about 10 vol. ppm. of water or less and most preferably about 5 vol. ppm. or less. If the water level in the hydrogen stream is too high, drying of same can be conveniently accomplished by contacting the hydrogen stream with a suitable desiccant such as those mentioned above.

In the reforming embodiment, an effluent stream is withdrawn from the reforming zone and passed through a cooling means to a separation zone, typically maintained at about 25° F. to 150° F., wherein a hydrogenrich gas stream is separated from a high octane liquid product stream, commonly called an unstabilized reformat. When the water level in the hydrogen stream is outside the range previously specified, at least a portion of this hydrogen-rich gas stream is withdrawn from the

separating zone and passed through an adsorption zone containing an adsorbent selective for water. The resultant substantially water-free hydrogen stream can then be recycled through suitable compressing means back to the reforming zone. The liquid phase from the separating zone is typically withdrawn and commonly treated in a fractionating system in order to adjust the butane concentration, thereby controlling front-end volatility of the resulting reformate.

The operating conditions utilized in the numerous hydrocarbon conversion embodiments of the present invention are in general those customarily used in the art for the particular reaction, or combination of reactions, that is to be effected. For instance, alkylaromatic, olefin, and paraffin isomerization conditions include: a 15 temperature of about 32° F. to about 1000° F. and preferably from about 75° F. to about 600° F., a pressure of atmospheric to about 100 atmospheres, a hydrogen to hydrocarbon mole ratio of about 0.5:1 to about 20:1, and an LHSV (calculated on the basis of equivalent liquid volume of the charge stock contacted with the catalyst per hour divided by the volume of conversion zone containing catalyst and expressed in units of hr.<sup>-1</sup>) of 20 about 0.2 to 10. Dehydrogenation conditions include: a 25 temperature of about 700° F. to about 1250° F., a pressure of about 0.1 to about 10 atmospheres, a liquid hourly space velocity of about 1 to 40, and a hydrogen to hydrocarbon mole ratio of about 1:1 to 20:1. Likewise, typical hydrocracking conditions include: a pressure of about 500 psig. to about 3000 psig., a temperature of about 400° F. to about 900° F., an LHSV of 30 about 0.1 to about 10, and hydrogen circulation rates of about 1000 to 10,000 SCF per barrel of charge.

In the reforming embodiment of the present invention, the pressure utilized is selected from the range of 35 about 0 psig. to about 1000 psig., with the preferred pressure being about 50 psig. to about 600 psig. Particularly good results are obtained at low or moderate pressure; namely, a pressure of about 100 to 450 psig. In fact, it is a singular advantage of the present invention that it allows stable operation at lower pressure than have heretofore been successfully utilized in so-called "continuous" reforming systems (i.e. reforming for periods of about 15 to about 200 or more barrels of charge per pound of catalyst without regeneration) with conventional sulfided platinum-rhenium catalyst systems. In other words, the sulfided superactive multimetallic catalyst of the present invention allowed the operation of a continuous reforming system to be conducted at lower pressure (i.e. 100 to about 350 psig.) for about the same 45 or better catalyst cycle life before regeneration as has been heretofore realized with conventional sulfided platinum-rhenium catalysts at higher pressure (i.e. 300 to 600 psig.).

The temperature required for reforming with the 55 instant catalyst is markedly lower than that required for a similar reforming operation using a high quality sulfided platinum-rhenium catalyst of the prior art. This significant and desirable feature of the present invention is a consequence of the superior activity of the sulfided superactive multimetallic catalyst of the present invention for the octane-upgrading reactions that are preferably induced in a typical reforming operation. Hence, the present invention requires a temperature in the range of from about 775° F. to about 1100° F. and preferably 60 about 850° F. to about 1050° F. As is well known to those skilled in the continuous reforming art, the initial selection of the temperature within this broad range is

made primarily as a function of the desired octane of the product reformate considering the characteristics of the charge stock and of the catalyst. Ordinarily, the temperature then is thereafter slowly increased during the run to compensate for the inevitable deactivation that occurs to provide a constant octane product. Due to the outstanding initial activity of the catalyst of the present invention, not only is the initial temperature requirement lower, but also the average temperature requirement

used to maintain a constant octane product is, for the instant catalyst system, substantially better than for an equivalent operation with a high quality sulfided platinum-rhenium catalyst system of the prior art; for instance, a sulfided catalyst prepared in accordance with the teachings of U.S. Pat. No. 3,415,737. Moreover, it is a singular feature of the catalyst of the present invention that the average C<sub>5</sub>+ yield and the C<sub>5</sub>+ yield stability associated therewith can be markedly superior relative to those exhibited by this high quality bimetallic reforming catalyst of the prior art when both catalyst systems are run at equivalent severity levels. The superior activity, selectivity and stability characteristics of the instant catalyst can be utilized in a number of highly beneficial ways to enable increased performance of a catalytic reforming process relative to that obtained in a similar operation with a sulfided platinum-rhenium catalyst of the prior art, some of these are: (1) octane number of C<sub>5</sub>+ product can be increased without sacrificing average C<sub>5</sub>+ yield and/or catalyst run length; (2) the duration of the process operation (i.e. catalyst run length or cycle life) before regeneration becomes necessary can be increased; (3) C<sub>5</sub>+ yield can be increased by lowering average reactor pressure with no change in catalyst run length; (4) investment costs can be lowered without any sacrifice in cycle life or in C<sub>5</sub>+ yield by lowering recycle gas requirements thereby saving on capital cost for compressor capacity or by lowering initial catalyst loading requirements thereby saving on cost of catalyst and on capital cost of the reactors; and (5) throughout can be increased significantly at no sacrifice in catalyst cycle life or in C<sub>5</sub>+ yield if sufficient heater capacity is available.

The reforming embodiment of the present invention also typically utilizes sufficient hydrogen to provide an amount of about 1 to about 20 moles of hydrogen per mole of hydrocarbon entering the reforming zone, with excellent results being obtained when about 2 to about 6 moles of hydrogen are used per mole of hydrocarbon. Likewise, the liquid hourly space velocity (LHSV) used in reforming is selected from the range of about 0.1 to about 10, with a value in the range of about 1 to about 5 being preferred. In fact, it is a feature of the present invention that it allows operations to be conducted at higher LHSV than normally can be stably achieved in a continuous reforming process with a high quality sulfided platinum-rhenium reforming catalyst of the prior art. This last feature is of immense economic significance because it allows a continuous reforming process to operate at the same throughput level with less catalyst inventory or at greatly increased throughput level with the same catalyst inventory than that heretofore used with conventional sulfided platinum-rhenium reforming catalyst at no sacrifice in catalyst life before regeneration.

The following examples are given to illustrate further the preparation of the sulfided superactive multimetallic catalytic composite of the present invention and the use thereof in the conversion of hydrocarbons. It is under-

stood that the examples are intended to be illustrative rather than restrictive.

## EXAMPLE I

A sulfur-free alumina carrier material comprising 1/16 inch spheres was prepared by: forming an aluminum hydroxy chloride sol by dissolving substantially pure aluminum pellets in a hydrochloric acid solution, adding hexamethylenetetramine to the resulting alumina sol, gelling the resulting solution by dropping it into an oil bath to form spherical particles of an alumina-containing hydrogel, aging and washing the resulting particles and finally drying and calcining the aged and washed particles to form spherical particles of gamma-alumina containing about 0.3 wt. % combined chloride. Additional details as to this method of preparing the preferred gamma-alumina carrier material are given in the teachings of U.S. Pat. No. 2,620,314.

An aqueous sulfur-free impregnation solution containing chloroplatinic acid and hydrogen chloride was then prepared. The alumina carrier material was thereafter admixed with the impregnation solution. The amount of the metallic reagent contained in this impregnation solution was calculated to result in a final composite containing, on an elemental basis, 0.375 wt. % platinum. In order to insure uniform dispersion of the platinum component throughout the carrier material, the amount of hydrogen chloride used in this impregnation solution was about 2 wt. % of the alumina particles. This impregnation step was performed by adding the carrier material particles to the impregnation mixture with constant agitation. In addition, the volume of the solution was approximately the same as the bulk volume of the alumina carrier material particles so that all of the particles were immersed in the impregnation solution. The impregnation mixture was maintained in contact with the carrier material particles for a period of about  $\frac{1}{2}$  to about 3 hours at a temperature of about 70° F. Thereafter, the temperature of the impregnation mixture was raised to about 225° F. and the excess solution was evaporated in a period of about 1 hour. The resulting dried impregnated particles were then subjected to an oxidation treatment in a dry air stream at a temperature of about 975° F. and a GHSV of about 500 hr.  $^{-1}$  for about  $\frac{1}{2}$  hour. This oxidation step was designed to convert substantially all of the platinum ingredient to the corresponding platinum oxide form. The resulting oxidized spheres were subsequently contacted in a halogen treating step with an air stream containing H<sub>2</sub>O and HCl in a mole ratio of about 30:1 for about 2 hours at 975° F. and a GHSV of about 500 hr.  $^{-1}$  in order to adjust the halogen content of the catalyst particles to a value of about 1 wt. %. The halogen-treated spheres were thereafter subjected to a second oxidation step 55 with a dry air stream at 975° F. and a GHSV of 500 hr.  $^{-1}$  for an additional period of about  $\frac{1}{2}$  hour.

The resulting oxidized, halogen-treated, platinum-containing carrier material particles were then subjected to a dry reduction treatment designed to reduce substantially all of the platinum component to the elemental state and to maintain a uniform dispersion of this component in the carrier material. This reduction step was accomplished by contacting the particles with a hydrocarbon-free, dry hydrogen stream containing less 65 than 5 vol. ppm. H<sub>2</sub>O at a temperature of about 1050° F., a pressure slightly above atmospheric, a flow rate of hydrogen through the particles corresponding to a

GHSV of about 400 hr.  $^{-1}$  and for a period of about one hour.

A sulfur-containing rhenium carbonyl complex, [C<sub>6</sub>H<sub>5</sub>SRh(CO)<sub>3</sub>]<sub>3</sub>, was thereafter dissolved in an anhydrous acetone solvent in order to prepare the rhenium carbonyl solution which was used as the vehicle for reacting the rhenium carbonyl complex with the carrier material containing the uniformly dispersed platinum. The amount of this complex used was selected to result in a finished catalyst containing about 0.375 wt. % rhenium derived from rhenium carbonyl. The resulting rhenium carbonyl solution was then contacted under appropriate impregnation conditions with the reduced, platinum-containing alumina carrier material particles resulting from the previously described reduction step. The impregnation conditions utilized were: a contact time of about one half to about three hours, a temperature of about 70° F. and a pressure of about atmospheric. It is important to note that this impregnation step was conducted under a nitrogen blanket so that oxygen was excluded from the environment and also this step was performed under anhydrous conditions. Thereafter, the acetone solvent was removed under flowing nitrogen at a temperature of about 175° F. for a period of about one hour. The resulting dry rhenium carbonyl-impregnated particles were then subjected to a pyrolysis-sulfiding step designed to decompose the resulting rhenium carbonyl component and simultaneously to liberate a sulfiding agent. This step involved 20 subjecting the rhenium carbonyl-impregnated particles to a flowing hydrogen stream at a first temperature of about 230° F. for about one half hour at a GHSV of about 600 hr.  $^{-1}$  and at atmospheric pressure. Thereafter, in the second portion of the pyrolysis-sulfiding step 25 the temperature of the impregnated particles was raised to about 575° F. for an additional interval of about one hour until the evolution of CO was no longer evident. During the course of this step, a sulfiding agent was liberated in situ and thereafter immediately contacted 30 with the catalyst particles at conditions which facilitated the sulfiding of this catalyst system as was manifest by a sulfur analysis performed on the resulting catalyst particles which showed they picked up about 0.044 wt. % sulfur, calculated on an elemental basis.

A sample of the resulting sulfided and pyrolyzed rhenium-carbonyl- and platinum-containing catalytic composite contained, on an elemental basis, about 0.375 wt. % platinum, about 0.375 wt. % rhenium derived from the carbonyl, about 1.0 wt. % chlorine, and about 50 0.044 wt. % sulfur. The resulting catalyst is hereinafter referred to as Catalyst A. For this catalyst, the atomic ratio of rhenium to platinum was about 1.05:1 and the atomic ratio of sulfur to platinum was about 0.72:1.

## EXAMPLE II

In order to compare the sulfided superactive acidic multimetallic catalytic composite of the present invention with the platinum-rhenium-carbonyl catalyst system disclosed in my prior application Ser. No. 833,332 in a manner calculated to bring out the beneficial effects of sulfiding this catalyst system, a comparison test was made between the catalyst of the present invention prepared in accordance with Example I, Catalyst A, and a control catalyst, which it is to be emphasized is not a prior art catalyst system but is rather my prior invention as fully disclosed in my prior application Ser. No. 833,332. The control catalyst is hereinafter called Catalyst B and was manufactured according to the

procedure given in Example I except that the sulfiding step was omitted. This control catalyst contained these metals in the same amounts as the catalyst of the present invention; that is, the catalyst contained, on an elemental basis, about 0.375 wt. % platinum, about 0.375 wt. % rhenium, derived from rhenium carbonyl, and about 1.0 wt. % chlorine.

These catalysts were then separately subjected to a high stress accelerated catalytic reforming evaluation test designed to determine in a relatively short period of time their relative activity, selectivity, and stability characteristics in a process for reforming a relatively low-octane gasoline fraction. In all tests the same charge stock was utilized and its pertinent characteristics are set forth in Table I.

This accelerated reforming test was specifically designed to determine in a very short period of time whether the catalyst being evaluated has superior characteristics for use in a high severity reforming operation.

TABLE I

## Analysis of Charge Stock

|                           |      |
|---------------------------|------|
| Gravity, API at 60° F.    | 59.1 |
| Distillation Profile, °F. |      |
| Initial Boiling Point     | 210  |
| 5% Boiling Point          | 220  |
| 10% Boiling Point         | 230  |
| 30% Boiling Point         | 244  |
| 50% Boiling Point         | 278  |
| 70% Boiling Point         | 292  |
| 90% Boiling Point         | 316  |
| 95% Boiling Point         | 324  |
| End Boiling Point         | 356  |
| Chloride, wt. ppm.        | 0.2  |
| Nitrogen, wt. ppm.        | 0.1  |
| Sulfur, wt. ppm.          | 0.1  |
| Water, wt. ppm.           | 10   |
| Octane Number, F-1 clear  | 35.6 |
| Paraffins, vol. %         | 67.4 |
| Naphthenes, vol. %        | 23.1 |
| Aromatics, vol. %         | 9.5  |

Each run consisted of a series of evaluation periods of 24 hours, each of these periods comprises a 12-hour line-out period followed by a 12-hour test period during which the C<sub>5</sub>+ product reformate from the plant was collected and analyzed. The test runs for the Catalysts A and B were performed at identical conditions which comprises a LHSV of 2.0 hr.<sup>-1</sup>, a pressure of 300 psig., a 3.5:1 gas to oil ratio, and an inlet reactor temperature which was continuously adjusted throughout the test in order to achieve and maintain a C<sub>5</sub>+ target research octane of 100.

Both test runs were performed in a pilot plant scale reforming unit comprising a reactor containing a fixed bed of the catalyst undergoing evaluation, a hydrogen separation zone, a debutanizer column, and suitable heating means, pumping means, condensing means, compressing means, and the like conventional equipment. The flow scheme utilized in this plant involves commingling a hydrogen recycle stream with the charge stock and heating the resulting mixture to the desired conversion temperature. The heated mixture is then passed downflow into a reactor containing the catalyst undergoing evaluation as a stationary bed. An effluent stream is then withdrawn from the bottom of the reactor, cooled to about 55° F. and passed to a gas-liquid separation zone wherein a hydrogen-rich gaseous phase separates from a liquid hydrocarbon phase. A portion of the gaseous phase is then continuously passed through a high surface area sodium scrubber and the

resulting substantially water-free and sulfur-free hydrogen-containing gas stream is returned to the reactor in order to supply the hydrogen recycle stream. The excess gaseous phase from the separation zone is recovered as the hydrogen-containing product stream (commonly called "excess recycle gas"). The liquid phase from the separation zone is withdrawn therefrom and passed to a debutanizer column wherein light ends (i.e. C<sub>1</sub> to C<sub>4</sub>) are taken overhead as debutanizer gas and C<sub>5</sub>+ reformate stream recovered as the principal bottom product.

The results of the separate tests performed on the sulfided superactive catalyst of the present invention, Catalysts A, and the control catalyst, Catalyst B, are presented in FIGS. 1, 2 and 3 as a function of time as measured in days on oil. FIG. 1 shows graphically the relationship between C<sub>5</sub>+ yields expressed as liquid volume percent (LV%) of the charge for each of the catalysts. FIG. 2 on the other hand plots the observed hydrogen purity in mole percent of the recycle gas stream for each of the catalysts. And finally, FIG. 3 tracks inlet reactor temperature necessary for each catalyst to achieve a target research octane number 100.

Referring now to the results of the comparison test presented in FIGS. 1, 2 and 3 for Catalysts A and B, it is immediately evident that the sulfided superactive multimetallic catalytic composite of the present invention substantially outperformed the platinum-rhenium control catalyst in the areas of average hydrogen production and average C<sub>5</sub>+ yield. Turning to FIG. 1, it can be ascertained that the average C<sub>5</sub>+ selectivity for Catalyst A was clearly superior to that exhibited for Catalyst B with equivalent yield stability. The difference in C<sub>5</sub>+ yield averaged about 3 vol. % and it is clear evidence that Catalyst A has much better yield-octane characteristics than Catalyst B. Hydrogen selectivities for these two catalysts are given in FIG. 2 and it is clear from the data that there is a significant increase in hydrogen selectivity that accompanies the advance of the present invention; I attribute this increased hydrogen selectivity to the moderating effect of sulfur on the increased metal activity enabled by my unique platinum-rhenium catalyst system. The data presented in FIG. 3 immediately highlights the surprising and significant difference in activity between the two catalyst systems. From the data presented in FIG. 3, it is clear that Catalyst B was consistently about 40° to 45° F. more active than Catalyst A when the two catalysts were run at exactly the same conditions. The judicious use of the proper amount of a sulfur component in the case of my catalyst system, consequently, provides a convenient means to trade-off activity for superior C<sub>5</sub>+ yield and hydrogen production and allows my superactivated platinum-rhenium catalyst system to be precisely moderated in order to adjust the surprising characteristics of this unique catalyst system to applications where superior C<sub>5</sub>+ yield and hydrogen selectivity are more important than extremely high activity.

In final analysis, it is clear from the data presented in FIGS. 1, 2 and 3 for Catalysts A and B that the use of a sulfur component to interact with a platinum-rhenium catalyst system of the type shown in my prior application Ser. No. 833,332 provides an efficient and effective means for significantly promoting the C<sub>5</sub>+ and hydrogen selectivities of this catalyst system when it is utilized in a high severity reforming operation.

It is intended to cover by the following claims all changes and modifications of the above disclosure of the present invention which would be self-evident to a man of ordinary skill in the hydrocarbon conversion art or in the catalyst formulation art.

I claim as my invention:

1. A process for converting a hydrocarbon which comprises contacting said hydrocarbon at hydrocarbon conversion conditions with a catalytic composite comprising a sulfided combination of a catalytically effective amount of a pyrolyzed rhenium carbonyl component with a porous carrier material containing a uniform dispersion of catalytically effective amounts of a platinum group component which is maintained in the elemental metallic state during the incorporation and pyrolysis of the rhenium carbonyl component.

2. The process as defined in claim 1 wherein the platinum group component is platinum.

3. The process as defined in claim 1 wherein the platinum group component is ruthenium.

4. The process as defined in claim 1 wherein the platinum group component is rhodium.

5. The process as defined in claim 1 wherein the platinum group component is iridium.

6. The process as defined in claim 1 wherein the porous carrier material contains a catalytically effective amount of a halogen component.

7. The process as defined in claim 6 wherein the halogen component is combined chlorine.

8. The process as defined in claim 1 wherein the porous carrier material is a refractory inorganic oxide.

9. The process as defined in claim 8 wherein the refractory inorganic oxide is alumina.

10. The process as defined in claim 1 wherein the composite contains the components in an amount, calculated on an elemental metallic basis, corresponding to about 0.01 to about 2 wt. % platinum group metal, about 0.01 to about 5 wt. % rhenium and about 0.001 to about 0.2 wt. % sulfur.

11. The process as defined in claim 6 wherein the halogen component is present therein in an amount sufficient to result in the composite containing, on an elemental basis, about 0.1 to about 3.5 wt. % halogen.

12. The process as defined in claim 6 wherein the composite contains, on an elemental basis, about 0.05 to about 1 wt. % platinum group metal, about 0.05 to about 1 wt. % rhenium, about 0.5 to about 1.5 wt. % halogen and about 0.005 to about 0.1 wt. % sulfur.

13. The process as defined in claim 1 wherein the composite is prepared by the steps of: (a) reacting a sulfur-containing rhenium carbonyl complex with a porous carrier material containing a uniform dispersion of a platinum group component maintained in the elemental metallic state; (b) subjecting the resulting reac-

tion product to pyrolysis conditions selected to decompose the resulting rhenium carbonyl component and to thereby liberate a sulfiding agent, and (c) contacting the pyrolyzed product of step (b) with said sulfiding agent at sulfiding conditions.

14. The process as defined in claim 13 wherein the pyrolysis step is conducted under anhydrous conditions and in the substantial absence of free oxygen.

15. A process for converting a hydrocarbon as defined in claim 1 wherein the contacting of the hydrocarbon with the catalytic composite is performed in the presence of hydrogen.

16. A process as defined in claim 1 wherein the sulfided state of the catalytic composite is maintained during use in the conversion of hydrocarbons by continuously adding thereto a sulfiding agent in an amount sufficient to provide about 1 to about 500 wt. ppm. of the hydrocarbon charge.

17. The process as defined in claim 1 wherein the hydrogen conversion comprises reforming, the hydrocarbon comprises a gasoline fraction, the hydrocarbon conversion conditions comprise reforming conditions, and wherein said contacting is performed in the presence of hydrogen.

18. A process as defined in claim 17 wherein the reforming conditions include a temperature of about 700° to about 1100° F., a pressure of about 0 to about 1000 psig., a liquid hourly space velocity of about 0.1 to about 10 hrs.<sup>-1</sup> and a mole ratio of hydrogen to hydrocarbon of about 1:1 to about 20:1.

19. A process as defined in claim 18 wherein the reforming conditions utilized include a pressure of about 50 to about 350 psig.

20. A process for converting a hydrocarbon which comprises contacting said hydrocarbon at hydrocarbon conversion conditions with a catalytic composite comprising the sulfided and pyrolyzed reaction product formed by reacting a catalytically effective amount of a rhenium carbonyl complex with a porous carrier material containing a uniform dispersion of a catalytically effective amount of a platinum group metal maintained in the elemental metallic state during the incorporation of the rhenium carbonyl component, subjecting the resulting reaction product to pyrolysis conditions selected to decompose the resulting rhenium carbonyl component, and thereafter, contacting the pyrolyzed reaction product with a sulfiding agent at sulfiding conditions.

21. The process as defined in claim 20 wherein the porous carrier material contains a catalytically effective amount of a halogen component.

22. The process as defined in claim 21 wherein the halogen component is combined chlorine.

\* \* \* \* \*